

Dec. 1, 1931.

W. L. MILLER

1,834,132

LEADING-IN CONDUCTOR

Filed Nov. 26, 1924

Fig. 1.



Fig. 2.



Fig. 3.



Fig. 4.



WITNESSES:

*C. J. Weller*

*S. M. Pineda*

INVENTOR

*William L. Miller.*

BY

*Wesley G. Barr*  
ATTORNEY

## UNITED STATES PATENT OFFICE

WILLIAM L. MILLER, OF PITTSBURGH, PENNSYLVANIA, ASSIGNOR TO WESTINGHOUSE ELECTRIC & MANUFACTURING COMPANY, A CORPORATION OF PENNSYLVANIA

## LEADING-IN CONDUCTOR

Application filed November 26, 1924. Serial No. 752,365.

My invention relates to leading-in conductors for evacuated electrical discharge devices and it has particular relation to the joint between a flexible terminal conductor and the leading-in wire which is sealed into the glass vessel of such devices.

One object of my invention is to provide a stiffening means for the end of a flexible terminal wire in order to improve the joint 10 between the same and a substantially rigid conductor which is sealed into the glass vessel of an evacuated discharge device.

Another object of my invention is to provide an improved process and the resultant 15 structure, relating to a joint between a rigid leading-in conductor, of tungsten or other material suitable for glass seals, and a flexible terminal conductor, preferably of stranded copper wire, a ferrule being first clamped 20 around the end of the flexible conductor, and the latter being then joined to the lead-in wire, preferably by percussive welding.

More generally stated, an object of my invention is to provide a means and method of 25 improving the conductivity of a weld between a tungsten wire and a stranded copper wire, or other dissimilar wires, and to remove all bending stresses from the welded section.

In the accompanying drawings, 30 Figure 1 is a sectional view of a hot-cathode rectifier embodying my invention.

Fig. 2 is an enlarged view, similar to Fig. 1, illustrating, in detail, the joint between the flexible terminal conductor and the rigid 35 conductor which is sealed into the glass vessel,

Fig. 3 is a view, similar to Fig. 2, illustrating a step in the process of making my improved conductor, and

Fig. 4 is a view, similar to Fig. 2, illustrating a modification of my invention.

In Fig. 1, my invention is shown applied to an evacuated hot-cathode rectifier comprising a glass vessel 1 enclosing a cylinder anode 2 and an axially disposed incandescent cathode 3. The anode 2 is supported upon a leading-in wire 4 which is sealed into a re-entrant portion of the glass vessel. The cathode 3 is made of tungsten wire which is 50 mounted between two leading-in wires 5 and

6 which are also sealed into a re-entrant portion of the glass vessel.

In rectifiers of large capacity, the leading-in wires 4, 5 and 6, respectively, are usually made of tungsten, molybdenum or other metal which seals well into glass, and the leading-in wires are fairly thick, in order to carry the heavy currents involved. It is then necessary to join a flexible stranded copper wire 7 to the end portion of each of the 55 leading-in wires, since the rigid tungsten or molybdenum conductors are not well adapted for providing a direct connection with the base or any other terminals to which the electrodes of the device are to be connected. 60

Heretofore, the stranded flexible terminal wire has been soldered, brazed or welded directly to the rigid leading-in wire, and the joint between the two wires has been a source of trouble, on account of the difficulty in providing a strong mechanical joint between the two wires. In manipulating the flexible copper wire, the stresses transmitted to the joint have been too large, with the result that the copper wire has very often broken off at the 70 joint. 75

According to my invention, I so stiffen the end portion of the flexible wire near the joint that the stress incident to manipulation of the flexible wire is not fully transmitted to 80 the relatively weak point at which the two wires are joined together.

As shown in Fig. 2, the end portion of the stranded copper wire 7 is provided with a cylindrical ferrule 8, of nichrome or other 85 sheet metal, which is tightly clamped around the copper strands. The ferrule-capped copper wire is then welded to the rigid leading-in conductor 5 which is sealed into the glass. Thus, when the copper wire 7 is bent 90 sidewise, the ferrule 8 takes up a part of the strain and safeguards the joint.

The use of a ferrule for stiffening the end portion of the flexible copper wire is of particular importance when making the joint 95 between the two wires by the percussive welding process. In carrying out the last-mentioned process, the two wires are connected in a circuit including a source of electrical energy, such as a charged condenser, the 100

wires being first brought into contact, immediately separated, and thereupon moved through the path of the resulting arc to effect a percussive engagement of the molten ends. The manipulations involved in the process of percussively welding the flexible or stranded wire 7 and the rigid wire 5 are greatly facilitated by the use of a stiff sheet-metal ferrule surrounding the end portion 10 of the flexible conductor, as such a ferrule permits the welding of the two conductors in the same manner as if the conductors were both rigid. As is well known, the percussive method of welding wires produces joints 15 which are electrically and mechanically superior to other kinds of joints, and such welding is very difficult and expensive to carry out with an ordinary stranded, flexible conductor, owing to the tendency of the individual strands to become excessively heated and splutter. The stranded wire lacks, furthermore, the rigidity required in order to effect the percussive engagement.

The use of a ferrule or sleeve on the end 25 of the copper conductor has the further advantage that it prevents the copper, which has a much lower melting point than tungsten, from melting and falling away before the tungsten reaches a welding temperature.

30 When the weld is completed, the flexible conductor and the surrounding ferrule are both welded to the rigid leading-in wire in a single operation. I have obtained the best results when using a ferrule of nichrome in connection with a stranded copper wire and a leading-in wire of tungsten.

In Fig. 4 is shown a modification of my invention wherein the joint made according to my invention between the flexible conductor 40 7 and the rigid leading-in wire 5, is further strengthened by soldering additional metal 9 around the joint of the ferrule 8 and the rigid conductor 5.

In the claims, the expression "high temperature metal" means either tungsten or molybdenum.

I claim as my invention:

1. The method of uniting a copper conductor to a conductor of high-temperature metal which comprises placing a nichrome sleeve about the immediate end of said copper conductor and welding said immediate end to one end of said second-named conductor.

55 2. The method of uniting a copper conductor to a conductor of high-temperature metal which comprises placing a sleeve of material capable of fusing with both the copper and the high-temperature metal about the immediate end of said copper conductor and welding said immediate end to one end of said second-named conductor.

3. The method of welding a stranded copper conductor to a conductor of high-temperature metal which comprises placing a

nichrome sleeve about one end of said stranded conductor and substantially flush with said end, bringing said end and one end of said second-named conductor to a welding temperature, and pressing said ends together. 70

4. The method of welding a stranded copper conductor to a conductor of high-temperature metal which comprises placing a sleeve of material capable of fusing with both the copper and the high-temperature metal about one end of said stranded conductor and substantially flush with said end, bringing said end and one end of said second-named conductor to a welding temperature, and pressing said ends together. 75

80 5. The method of welding a stranded conductor to a solid conductor having a higher melting point than said stranded conductor which consists in applying a metal sleeve or ferrule about the immediate end of said stranded conductor, said sleeve having a higher melting point than said stranded conductor, and then welding said sleeve and said immediate end to one end of said solid conductor. 85

90 6. The method of welding a flexible conductor to a rigid conductor having a higher melting point than said flexible conductor which comprises placing a metal sleeve or ferrule about the immediate end of said flexible conductor, said sleeve having a higher melting point than said flexible conductor, bringing said immediate end and one end of said rigid conductor to a welding temperature, and then pressing said ends together. 95

100 7. A composite body consisting of a flexible metallic conductor, a reinforcing metallic sleeve positioned about the immediate end of said flexible conductor, and a rigid metallic conductor having one end thereof joined by fusion to both said flexible conductor and said sleeve. 105

110 8. A composite body consisting of a stranded metallic conductor, a reinforcing metallic sleeve positioned about the immediate end of said stranded conductor, and a rigid metallic conductor having one end thereof joined by fusion to both said stranded conductor and said sleeve.

115 9. A composite body consisting of a flexible metallic conductor, a reinforcing metallic member positioned about the immediate end of said flexible conductor, and a rigid metallic conductor having one end thereof joined by fusion to both said flexible conductor and said member. 120

In testimony whereof, I have hereunto subscribed my name this 18th day of Nov., 1924.

WILLIAM L. MILLER.

125

130